

No. 781,935.

PATENTED FEB. 7, 1905.

L. CLARK.  
LEAF FOR BOOKS.  
APPLICATION FILED NOV. 14, 1903.



Witnesses:

John Enders,  
Geo. C. Dawson

Inventor  
Lincoln Clark,  
By Dyrnford Dyrnford & Lee,  
Att'y.

## UNITED STATES PATENT OFFICE.

LINCOLN CLARK, OF CHICAGO, ILLINOIS, ASSIGNOR OF TWO-THIRDS TO  
W. GIFFORD JONES AND HARRY S. JONES, OF CHICAGO, ILLINOIS.

## LEAF FOR BOOKS.

SPECIFICATION forming part of Letters Patent No. 781,935, dated February 7, 1905.

Application filed November 14, 1903. Serial No. 181,199.

*To all whom it may concern:*

Be it known that I, LINCOLN CLARK, a citizen of the United States, residing at Chicago, in the county of Cook and State of Illinois, 5 have invented a new and useful Improved Leaf for Books, of which the following is a specification.

My invention relates to improvements in the sized-paper sheets forming the leaves of books, and more particularly those of loose-leaf ledgers.

It is desirable to provide, particularly for account-books, leaves which will tend normally to lie flatwise upon each other when the 15 books are open to present firm surfaces to the pen, and a common manner of forming such leaves is to cause an area or zone of each sheet adjacent to its binding edge to be more flexible than the other parts of the sheet. Various 20 methods have been employed for providing the said flexible zones or areas; but they all, so far as I am aware, involve treatments or operations which are more laborious or expensive than is thought to be desirable and in 25 those constructions which have proven the most practical heretofore tend materially to weaken the paper along well-defined lines, whereby, particularly after frequent turning of the leaves, and consequent flexing along 30 those lines, the leaves tend to become too weak thereat to withstand ordinary handling.

My object is to provide a new and improved method of rendering flexible without materially weakening areas or zones on sized-paper 35 sheets; and my invention consists in the method I employ and also in the improved leaves produced by the said method.

In the accompanying drawings, Figure 1 is a plan view of a loose leaf provided in accordance with my invention; Fig. 2, an edge view of the same, and Fig. 3 also an edge view showing the leaf bent under its own weight at the zone of greatest flexibility.

A represents a sheet of calendered paper 45 having a binding-edge portion *a*. In carrying out my invention I subject the leaf between, for example, the dotted lines *b b* to a mechanical flexing operation which consists, preferably, in turning the paper upon itself

and varying the place of curvature by relative movement of the parts of the paper to weaken or fracture the sizing coating throughout the band portion *c* defined by said dotted lines. This flexing operation may be repeated as often as necessary; but ordinarily the 55 desired result may be obtained by folding the paper to curve the same about an almost infinitesimal radius and varying the place of curvature until the desired area has been treated and finally reversing the direction of 60 curvature and varying the place of curvature until the same area has been flexed in the opposite direction. In the flexing operation sufficient pressure is applied to bend the paper closely upon itself, while the continuous 65 change in the place of curvature prevents the paper from being sharply folded or creased. The effect of the treatment is to thoroughly fracture the sizing coatings of the paper along almost infinitely close lines without injuring 70 the fiber of the paper, which commonly is of linen. At the same time the sizing coatings are left in such a smooth and complete condition as to enable the surfaces to be written upon freely with ink. Thus, it will be understood, the tenacity and smoothness of the treated section of the leaf are unimpaired, 75 while the flexibility is increased greatly. If desired, the paper may be bent over a wire or strip presenting a blunt rounded edge and 80 then drawn across the same to flex the paper without creasing it, while fracturing or weakening, the sizing coatings to decrease the resilience thereof. In the flexing operation uniformity of curvature coupled with continuity 85 of change of place of curvature is desirable to avoid the production of creases, which would unduly weaken the sheet along definite lines.

Rendering the paper highly flexible at the section operated upon in the manner described 90 does not materially change the appearance of the paper, and the desired result is attained without either thickening or thinning the paper at said section. Moreover, great uniformity of flexibility results from the improved treatment, and tests have shown that the tearing strength of the paper is practically unimpaired, attributable, as suggested above,

to the preservation of the fiber of the paper and the absence of definite lines of weakening. As the tenacity of the paper is practically unimpaired, the treated section may extend from 5 the extreme top to the bottom edge of the leaf.

In carrying out my method any kind of ledger-paper may be provided with a bending zone without regard to the thickness of the paper, unevennesses in the surface, or the 10 state of the paper with regard to dryness.

Changes within the spirit of my invention are contemplated. Hence no undue limitation should be understood from the foregoing detailed description.

15 What I regard as new, and desire to secure by Letters Patent, is—

1. The method of treating sized paper to render it more flexible over a limited bending area, which consists in minutely fracturing 20 the sizing coating by flexing the sheet uniformly throughout a band portion only without scoring or creasing, whereby the fiber of said band portion is left uninjured, definite lines of weakness avoided therein and the surfaces thereof preserved for writing purposes, the remainder of the paper being left unchanged in all its qualities, for the purpose 25 set forth.

2. The method of treating sized paper to 30 render it more flexible over a limited bending area, which consists in minutely fracturing the sizing coating by subjecting the leaf to a flexing operation throughout a limited area only and varying the place of curvature uniformly throughout said area, without scoring 35 or creasing, whereby the fiber of the paper at said area is left uninjured, definite lines of weakness thereat avoided and the surfaces thereof preserved for writing purposes, the 40 remainder of the paper being left unchanged in all its qualities, for the purpose set forth.

3. The method of treating sized paper to render it more flexible over a limited bending area, which consists in minutely fracturing 45 the sizing coating by subjecting the leaf to a

flexing operation throughout a limited area only and varying the place of curvature uniformly throughout said area, and then reversing the direction of curvature and varying the place of curvature uniformly throughout said 50 area, without creasing or scoring, whereby the fiber of the paper at said area is left uninjured, definite lines of weakness thereat avoided and the surfaces thereof preserved for writing purposes, the remainder of the paper being left unchanged in all its qualities for the purpose 55 set forth.

4. As a new article of manufacture, a leaf of sized book-paper having a transverse band portion adjacent to its binding margin with 60 the sizing coatings minutely fractured uniformly throughout said band portion, said band portion retaining its fiber and surfaces practically unimpaired and possessing greatly-increased flexibility, the remainder of the paper retaining its original qualities, substantially 65 as and for the purpose set forth.

5. The method of treating a leaf of sized book-paper, to provide a zone of increased flexibility, which consists in minutely fracturing the sizing coatings by subjecting a band portion parallel with and adjacent to the binding edge of the leaf to a flexing operation and varying the place of curvature uniformly parallel with said binding edge throughout said 75 band portion, and then reversing the direction of curvature and varying the place of curvature uniformly throughout said band portion, whereby the fiber at said band portion is left uninjured and definite lines of weakness avoided, the flexibility thereat increased, and the surfaces thereof preserved for writing purposes, the remainder of the leaf being left unchanged in all its qualities, substantially as 80 and for the purpose set forth.

LINCOLN CLARK.

In presence of—

WALTER N. WINBERG,  
F. M. WIRTZ.